

## UNITED STATES PATENT OFFICE.

GUILLERMO ARIS, OF BARCELONA, SPAIN.

## DYEING AND PRINTING WITH PHENYLAMINE BLACK.

No Drawing. Application filed February 16, 1922, Serial No. 537,087, and in Spain March 1, 1921.

My invention relates to the dyeing and printing of textile fibres with aniline black and the object of the invention is an improved process by which a considerable economy is effected in the dyeing and printing over the methods hitherto employed.

My invention consists essentially in adding to the dyeing bath or to the printing bath, a small quantity of an azo-derivative of ordinary aniline oil or of any one of its components or methylation, etc., derivatives. The presence of this small quantity of azo-derivative greatly increases the affinity between the color and the fibres, so that it is possible to obtain a fixed intensity of black, while using smaller quantities of aniline oil and auxiliary chemicals than with the method usually employed. These azo-derivatives are products so cheap that the cost of the small quantity employed in this invention is negligible.

To carry out my invention the base may be prepared using instead of the ordinary aniline oil, aniline oil, containing a small proportion of an azo-derivative of the same, or adding to the composition of the dyeing or printing bath the necessary proportion of an azo-derivative of industrial aniline.

The chief component of the base, that is to say industrial aniline oil, is not pure but it generally contains toluidines and xylydines; therefore the azo-derivative employed may be not only an azo-derivative of the aniline, but may also contain the azo-derivatives of toluidine or xylydine as well as an azo-derivative of any of those substances obtained by sulphonation, methylation or by the introduction of groups belonging to another order, into the anilin.

These azo-derivatives may be of an acid, basic or neutral character, being all of them distinguished by the general azo-linkage— $N=N-$ .

In carrying out my invention, I may employ any of the known metallic compounds for transferring or carrying oxygen but a greater economy is obtained by using as oxygen-transferring agent the ferrous chloride,  $FeCl_2$ , either alone or associated with volatile compounds.

Very many azo-derivatives may be used to carry out this process. The following examples are mentioned:

Azo-derivatives from aniline



Azobenzene,



Azobenzoic acid,



Azophenylene,



Hydrazobenzene,



Diazo-amido-benzene,



Amido-azo-benzene,



Azo-oxy-benzene,



and their derivatives by methylation or by introduction of groups belonging to another order.

Azo-derivatives of toluidine may also be used. They are homologous compounds of the above mentioned bases, where the group  $C_6H_5$  is substituted by  $C_5H_4CH_3$ .

Azo-derivatives of xylydine and their isomers and derivatives. They are homologous compounds of the first above mentioned series where the group  $C_6H_5$  is substituted by  $C_6H_3(CH_3)_2$ .

The quantity of azo-derivative which is necessary in order to produce the above-mentioned increase of affinity is very small; it does not amount to 2% of the quantity of aniline to be employed and since practically those compounds cost not much more than aniline, their price does not materially affect the total cost of the dyeing process.

The most appropriate vehicle for the application of azo-derivatives for black oxidation is industrial aniline oil. By the pre-

55

60

65

70

75

80

95

100

vious manufacture or preparation of aniline oil containing one of its azo-derivatives, much better solution is obtained, this being an indispensable condition for maximum efficiency. This aniline oil containing its azo-derivative in the state of intimate solution I call azo-oil.

This may contain the azo-derivative in the exact and necessary proportion (less than 10 2% according to the selected derivative) for acting directly as a component of the baths or dyeing pastes, or it may contain a larger quantity of it, and in this case it must be diluted with aniline oil in order to produce 15 an azo-oil of the concentration suitable for operating with it either in dyeing or printing or for adding that diluting aniline separately.

In this invention the composition of the 20 baths for dyeing or printing with an azo-derivative is not solely characterized by the ingredients it contains. It is also characterized by the appearance shown by the products employed which are characterized by the yellow color of azo-derivatives of anilines, toluidines and xylidines; and it is likewise characterized by the aspect of the material that is to be dyed or printed during the course of the manufacture.

With the usual baths, when not much used or when recently prepared, the material on 30 being impregnated with ordinary aniline-black remains white or a dirty white, or a slightly greenish if made with black prussiate, and so it remains until oxidation begins. In printing it is usual to add an auxiliary color (methyl-violet, for instance) in order to render the printing visible on being done.

With aniline-black with the addition of 40 azo-derivatives the dyed or printed material is of yellow-color, and has the peculiarity that before oxidation begins (before assuming the emerald green color) it shows a characteristic vivid pink color. The azo-oil (whatever its concentration may be) as well as the dyeing baths or printing pastes, dye textile fibres or the human skin (so that it can be tested for instance on one's hand) a 50 yellow color turning into light red or vivid pink by the action of an acid (hydrochloric acid, for instance).

When applying this invention it is not necessary to modify any of the apparatus 55 already in use in the industry and the manipulations need not be changed.

In printing, powerful washing machines may be dispensed with, because in the most delicate case, that of designs surcharged on 60 a white ground, with a simple washing of the fabric (spread to its full width) after the bath of bichromate, very pure whites are obtained.

With the presence of azo-derivatives, all 65 the aniline present in the dyeing or print-

ing bath is transformed into black fixed on the fibre. This explains the purity of the white which are obtained directly without requiring strong washing.

In the dyeing of pieces in the "foulard" 70 manner, it is advisable to dissolve all the products in water containing about six grams per litre of starch, gum mucilage or analogous compositions with the object of giving more stability to the solution. 75

I shall now discuss the improvements of aniline-black oxidation due, as stated in the beginning, to the employment of chloride of iron  $FeCl_2$  as the oxygen-transferring agent. This compound has already been 80 proposed for producing black-oxidation, but it has not been adopted in industrial practice, notwithstanding all its advantages, because of its not having been used under favorable conditions and it has never been 85 used in presence of azo-derivatives of aniline and its homologues.

In printing, it has been employed in presence of excessive quantities of acid; this is, at 90 least a quantity of acid equal to that of aniline. Under these conditions the rapid oxidation of the fabric ("steam-black") cannot be brought about because the fibre becomes greatly deteriorated.

The present invention embraces the improvement of obtaining the aniline-black, employing chloride of iron  $FeCl_2$  as the oxygen-transferring agent; in the presence of azo-derivatives of industrial aniline and in direct printing, operating with basic salt of 100 aniline. Under these conditions and without employing any other fixed metallic compounds, blacks of excellent quality either in printing or in dyeing can be produced in the most economical manner. 105

When prussiates are employed a great quantity of alkaline salts, totally inert for oxidation, are formed in the midst of the dyeing preparation; therefore, the black-prussiate ought to be oxidized at a very high 110 and persistent temperature. This does not occur when chloride of iron is used instead of prussiate. For this reason the oxidation of the black is possible at a lower temperature and more rapidly. The oxidation is 115 also deeper, thus saving in super-oxidizer later on.

Throughout the claims, where the term "aniline" is used, I intend to cover thereby the homologues and substitution derivatives as above indicated. The term "industrial aniline" is used in its ordinary sense to include a mixture of amino benzene with its homologues amino toluene, amino xylene. 120

In the specification and in the claims, "basic compounds" or "basic salts" are terms used to designate aniline compounds into the composition of which only that quantity of acid enters which is not sufficient to form a neutral salt. In the present case the quan- 125 130

ity of acid necessary to form these basic compounds is half of the acid theoretically required to form a neutral salt.

I claim:

5. 1. In the art of dyeing with anilin black, the step of treating the textile to be dyed, with a bath containing both anilin and an azo aromatic compound, the latter being present in amount not substantially over 10 2% of the former.
2. In the process of claim 1, the step of treating the textile with a mixture of industrial anilin and an azo compound derived therefrom.
15. 3. In the process of dyeing or printing with anilin black, treating the textile with a bath containing anilin, a small amount of an azo aromatic body and hydrochloric acid, the amount of the latter being only sufficient to form basic compounds with the dye-stuff.
20. 4. In the production of aniline black on the fibres, the addition to the anilin bath of a small quantity of an azo-derivative from industrial anilin, and conducting the operation in the presence of iron chloride as an oxygen-transferring agent.
25. 5. In the production of aniline black on the fibre, the process which comprises applying to the fibre a composition containing aniline, aniline hydrochloride, an azo-derivative of an aromatic amino compound of the benzene series, and an oxygen-transferring agent.
30. 6. In the production of aniline black on the fibre, the process which comprises applying to the fibre aniline oil with which has been incorporated an azo-derivative of an aromatic amino compound of the benzene series.
35. 7. In the dyeing of textile fibres with
40. aniline black, a dyeing bath comprising, instead of the usual anilne oil mixture, anilne oil with which has been incorporated an oxygen-transferring agent and less than 45 2%, based on the anilne present, of an azo-derivative of a constituent of industrial anilne oil.
45. 8. In the printing of fabrics with anilne black, a printing paste comprising, instead of the usual anilne oil, an anilne oil in which has previously been incorporated both ferrous chloride as an oxygen-transferring agent, and less than 2% of an azo-derivative of a constituent of industrial anilne oil. 50
50. 9. In the production of anilne black on the fibre, the process which comprises applying to the fibre anilne hydrochloride with which has been incorporated ferrous chloride and an azo-derivative of an aromatic amino compound of the benzene series. 55
55. 10. A composition suitable for use in the production of anilne black on the fibre, comprising anilne hydrochloride, an oxygen-transferring agent, and an azo-derivative of an aromatic amino compound of the benzene series. 60
60. 11. A composition as defined in claim 10 in which the oxygen-transferring agent is 65 ferrous chloride.
65. 12. A composition as defined in claim 10 in which the azo-derivative is an azo-benzene.
70. 13. A composition suitable for use in the production of anilne black on the fibre, comprising anilne, anilne hydrochloride, ferrous chloride, and an azo-derivative of anilne. 75

In testimony whereof I affix my signature

GUILLERMO ARIS.